

Feb. 23, 1971

R. T. EDDINGER ET AL

**3,565,766**

## COPYROLYSIS OF COAL AND HEAVY CARBONACEOUS RESIDUE

Filed Jan. 24, 1969

2 Sheets-Sheet 1

## HIGH VOLATILE B BITUMINOUS COAL



FIG. I.

INVENTORS  
RALPH TRACY EDDINGER  
JOHN F. JONES  
BY *Robert D. Jackson*  
*George E. Jones*  
*Milton Fischer*

Feb. 23, 1971

R. T. EDDINGER ET AL

3,565,766

COPYROLYSIS OF COAL AND HEAVY CARBONACEOUS RESIDUE

Filed Jan. 24, 1969

2 Sheets-Sheet 2

HIGH VOLATILE C BITUMINOUS COAL



FIG. 2.

INVENTORS  
RALPH TRACY EDDINGER  
JOHN F. JONES  
BY *Robert D. Jackson*  
*Engine M. Lewis*  
*Milton Jordan*

1

3,565,766

## COPYROLYSIS OF COAL AND HEAVY CARBONACEOUS RESIDUE

Ralph Tracy Eddinger, Princeton Junction, and John F. Jones, Princeton, N.J., assignors, by mesne assignments, to the United States of America as represented by the Secretary of the Interior

Filed Jan. 24, 1969, Ser. No. 793,735

Int. Cl. C10b 49/22, 55/10

U.S. Cl. 201—23

5 Claims

### ABSTRACT OF THE DISCLOSURE

Heavy hydrocarbonaceous residues are upgraded to lighter fractions by copyrolyzing them with coal particles—previously heated to remove from about 1% to about 10% volatiles therefrom—in the fluidized state, at a temperature between about 850° F., and about 1100° F. and recovering the resultant oily distillates and carbonaceous residues.

### BACKGROUND OF THE INVENTION

#### (A) Field of the invention

This invention relates to the processing of hydrocarbonaceous materials. More particularly, the invention pertains to the upgrading, to lower boiling products, of heavy hydrocarbon oils of the type recovered from petroleum, oil shale, tar sands, and coal refining.

#### (B) Description of the prior art

The treatment of heavy hydrocarbonaceous residues for the purposes of converting them to more valuable lighter fractions is well known in the refinery art. Commonly, the conversion is effected by the so-called delayed coking process wherein the residues are heated in a coking vessel, thereby forming lower boiling hydrocarbon fractions and a residue of bulk coke. More recently the coking has been performed in a fluidized bed. This is more efficient than delayed coking and moreover produces coke in powder rather than massive form.

It is also known to upgrade coal by heating it to form valuable oils. The basic procedure is to pyrolyze coal in a coking vessel and recover the oil distillate and carbonized residue or coke. Considerable improvements in the technology have been made and in this connection reference is made to U.S.P. 3,375,175 to Eddinger et al. In this process coal is pyrolyzed in a series of fluidized beds, in which the temperature of each succeeding stage is increased until essentially all volatiles have been evolved. The devolatilized, finely divided char residue is a valuable and useful carbonaceous byproduct.

### SUMMARY OF THE INVENTION

It has now been discovered that a heavy hydrocarbonaceous residue can be upgraded to yield lower boiling fractions by the fluidized copyrolysis of the residue with coal particles—previously heated until about 1-10% volatiles have been removed therefrom—for a time sufficient to remove all of the volatiles from the coal and residue condensable to oily liquids and recovering said oily liquids, product char and gas.

### DESCRIPTION OF THE INVENTION AND THE PREFERRED EMBODIMENTS

According to the present invention, generally satisfactory results are realized by introducing the heavy hydrocarbonaceous residue into the appropriate stage of a multistage coal pyrolysis system of the type disclosed in the aforesaid patent. The Eddinger et al. process provides for the carbonization to be performed in the absence of

2

added oxygen, thereby favoring maximum production of tar. In the Eddinger et al. process of coal pyrolysis, finely divided coal is heated at low pressures in a plurality of fluidized beds at successively higher temperatures, the result of which is to bring about an increase in yield of oily liquids recoverable from the coal. In general, the process comprises the steps of:

(1) In a first stage, heating the finely divided coal below its fusion temperature under oxygen-free conditions in a first fluidized bed formed by passing an inert gasiform stream upwardly through the stage to maintain the coal in the fluidized state until about 1% to about 10% of the coal volatiles have been removed as overheads and recovering oily liquids from said overheads,

(2) In at least a second stage, passing the so-treated coal into at least one other fluidized bed which is fluidized by the gaseous overheads from the subsequent stages at a temperature above that of the first bed and below the fusion point of the solids fed to that stage, under oxygen-free conditions, for a time sufficient to remove nearly all of the volatiles from the coal condensable to oily liquids.

(3) In a final stage passing, the thus-treated coal into a final fluidized bed which is fluidized by an oxygen-containing gas at a still higher temperature, to substantially devolatilize the coal, and

(4) Recovering the oily liquids from all stages subsequent to the first stage from the overheads of the second stage.

In practicing the invention, the hydrocarbonaceous residue in particulate form is introduced into a carbonization stage which follows the first stage of the Eddinger et al. process. Where the coal is carbonized in a series of stages, the hydrocarbonaceous material can be introduced at any one of the stages or combination of them. Both the hydrocarbonaceous material and coal undergo mutual carbonization in the presence of one another, resulting in the production of oily liquids and product char, in essentially the manner as when the coal alone is subjected to the same treatment. That is to say, the presence of the hydrocarbonaceous material in no way interferes with normal operation of the multistage coal pyrolysis. This is surprising since the presence of hydrocarbonaceous materials would be expected to cause severe coalescence of the coal particles during carbonization with concomitant loss of fluidization. Apparently the prepyrolysis of the coal particles in the first stage greatly diminishes their agglomeration tendencies to such an unexpected extent that they can tolerate the presence of the oily particles of the hydrocarbonaceous material.

A further advantage which is realized from the invention is a marked reduction in the loss of coal fines from the fluidized beds.

The hydrocarbonaceous material is conveniently introduced into the coal pyrolysis stages in the form of an atomized spray. This can readily be effected by heating the material to increase its fluidity, whereby it can be pumped and sprayed into the reaction vessel where the coal is being carbonized. Such hydrocarbonaceous materials represent the heavy residues left over from petroleum, oil shale, tar sands, and coal refining operations; they are available in a number of grades and types. A familiar class of these materials is the heavy residue remaining from atmospheric or vacuum crude distillation in the refining of petroleum. It is readily upgraded to valuable light fractions by the process of the invention. Other types of hydrocarbonaceous residues give comparable results.

The ratio of hydrocarbonaceous materials to coal will of course vary with a particular type of coal being subjected to pyrolysis. The ratio will also vary with the type of hydrocarbonaceous material being processed. Gener-

ally speaking however, we have ascertained that ratios in the neighborhood of 1:1 up to about 4:1 of coal by hydrocarbonaceous residue are readily processed in the manner of the present invention. By using high volatile C bituminous or subbituminous coals wherein the second-stage coal carbonization reactor temperature is above 900° F., operation with variable feed concentrations is feasible. Where the residue is premixed with char from the first stage before injection into the second stage, the char is more readily transported into the second-stage reactor at the lower ratio 2 parts coal, 1 part of residue. On the other hand, when operating with high volatile B bituminous coal, preferable ratios of coal to oil are 3 or 4. This is a consequence of the second-stage reactor being operated below 900° F. At this temperature the more refractory-type of residue does not undergo sufficient thermal cracking and vaporization to permit operability of the fluidized bed. The oil tends to ball up the char particles in the bed whereby fluidization cannot be maintained. When injecting the more refractory residue into the third stage at the lower coal to oil ratios, there appears to be a partial condensation of the residue vapors in the preceding second stage causing operating problems. Under these conditions, 4 to 1 ratio is preferred over 3 to 1 ratio. Accordingly, it has been our finding that the preferred ratio of coal to residuum is about 3 or 4 to 1, the type of coal tending to be the deciding factor. Preferably, the residue is introduced into a stage at a temperature above 900° F. with 950° F. being preferred. Temperatures below 900° F. generally produce poor results. Operating at temperatures above 1000° F. tends to form more gas and coke, at the expense of liquid yield. Here again, the particular type of coal being processed is the deciding factor on these temperature ranges. A small quality control run with a particular coal and residue will readily determine the optimum set of temperatures and conditions. In general, the pressure and residence times fall within the ranges set forth in the previously cited U.S. patent to Eddinger et al.

The process herein can best be understood by reference to the accompanying drawings in which FIG. 1 is the flow sheet of our process as applied to high volatile B bituminous coal with char recycle using petroleum residuum as the hydrocarbonaceous residue. FIG. 2 is a flow sheet of our process as applied to high volatile C bituminous coal and petroleum residuum.

Referring to the drawings, FIG. 1 discloses the preferred mode of operation with high volatile B bituminous coal. The coal is first crushed to a size desirable for fluidization, generally -14 mesh, and is fed into a first fluidized bed where it is maintained at a temperature sufficiently below the fusion temperature of the coal to prevent the mass from fusing, but sufficiently high to remove substantial quantities of volatiles in addition to unbound water. In high volatile B bituminous coals, this range is from about 600° F. to about 650° F. Fluidization is by means of an inert gas, preferably hot, oxygen-free flue gas, which both heats and fluidizes, although external heating may be used. About 1% to 10% of the weight of the dry coal is removed as overhead during a residence time of from about 1 to 30 minutes; of this overhead, about half represents material condensable to oily hydrocarbon liquids.

The dried preheated coal and hot residuum can then be separately fed into the second stage, although preferably to the third stage, where the mixture is immediately heated to a higher temperature, but below the fusion point of the coal, to start driving out the bulk of volatiles from the coal and residuum. The fluidizing medium is for the sake of heat economy the overhead from the third stage and consists of gas plus condensables from that stage. Residence time is from 1 to 30 minutes—temperature from 800° F. to 900° F. The second stage overhead includes all the gas and condensables formed from the

combined pyrolysis of coal and residuum excluding that which comes out of the preheating stage. In general there is enough condensable hydrocarbon to yield a total of about 35% to 60% oily liquid based on the combined weight of the original dry coal and residuum. The amount of gas produced is a function of the manner in which the fourth stage is operated and can be varied from about 10% to about 30% by weight of the original coal and residuum. Char from the fourth stage will vary from about 35% to 60% by weight of the original coal and residuum reflecting both the treatment in the last stage and the ash level in the original coal. Alternatively the fluidizing medium may be any inert gas and external heating may be used. However, it is preferable to avoid oxygen-fed at this second stage if high oil yields are to be realized.

The partially devolatized char from stage 2 goes into a third stage in which further fluidized bed pyrolysis of the coal-residuum mixture is effected at temperatures of the order of 950° F. to 1050° F. The fluidizing medium is preferably the overhead of stage 4. After 1 to 30 minutes in this stage, the char contains little more than a percent or so of volatiles which are recoverable as liquid condensates. The char from stage 3 is fed into a fluidized calcination bed maintained at a temperature between 1500° F. and 1800° F. by internal combustion of the char by the gas fed into the reactor as a fluidizing medium which may be air or oxygen. The overhead goes into stage three to act as a fluidizing medium. It may contain a very small amount of condensables; otherwise its constituents are dependent on the amount of oxygen in the fluidizing gas, and total residence time in the bed, these factors together controlling the temperature and the composition of the gas discharged. Preferably residence times are from 1 to 30 minutes, and with high oxygen concentrations, to achieve a temperature of 1600° F. in the bed, and an exit gas with high concentrations of hydrogen and carbon monoxide.

Referring to FIG. 2, this discloses a preferred mode of operation with high volatile bituminous C coal and petroleum residuum. Generally, the process of FIG. 2 is conducted identically to that of FIG. 1, except the residuum can be admixed with char prior to injection into carbonization stages 2 or 3. Moreover, stage 2 of FIG. 2 is operated at a temperature of 950° F. to 1000° F. which is higher than that of FIG. 1.

In the following examples, the fluidized bed reactors consist of a series of hollow steel cylindrical vessels. The first stage serves to effect prepyrolysis of the particles wherein 1 to 10% volatiles are removed. Stages 2 and 3 where the main pyrolysis of residuum and coal takes place while stage 4 is the combustion and gas forming stage. The inside diameters of the stages are 18, 12, 10 and 8 inches, respectively. Approximately 100 pounds of material can be processed per hour.

The residuum previously heated to increase its fluidity, is pumped into a feed nozzle for injection into the requisite carbonization stage. The coal particle are produced in any convenient comminuting equipment such as a hammer mill.

Oxygen diluted with nitrogen, steam, or recycle gas for temperature control is used to fluidize the last stage and provides the heat required for all but the first stage, which is externally heated. The second and third stages are fluidized and receive heat from the off-gas of the next heater stage. A portion of the second stage heat requirements is supplied by hot re-cycled char from the third stage, and, similarly, the third stage by char from the fourth stage as needed. Alternatively, oxygen can be added to the third stage at some loss of oil yield. Using multi-stage fluidized beds rather than a single fluidized bed for the pyrolysis of bituminous coal and petroleum residuum has the advantage that caking coals can be continuously processed without agglomeration.

**5**  
**EXAMPLE 1**

High volatile bituminous C coal (McKinley coal from New Mexico) and petroleum residuum (a heavy hydrocarbonaceous material recovered from petroleum refining) was processed through the aforescribed fluidized bed reactors and as further shown in the flow sheet of FIG. 2.

The conditions of operation, together with the results obtained, are summarized in the following table:

TABLE I.—RUNS WITH MCKINLEY HIGH VOLATILE C BITUMINOUS COAL AND SHORT RESIDUUM

|                                    | Run   |      |       |       |
|------------------------------------|-------|------|-------|-------|
|                                    | 1     | 2    | 3     | 4     |
| Dry coal weight <sup>1</sup>       | 100   | 100  | 100   | 100   |
| Short residuum weight <sup>1</sup> | 50    | 38   | 58    |       |
| Product yield distribution:        |       |      |       |       |
| Char weight <sup>1</sup>           | 55.2  | 2.9  | 60.9  | 65.0  |
| Oil weight <sup>1</sup>            | 18.5  | 34.8 | 45.1  | 62.2  |
| Gas weight <sup>1</sup>            | 15.8  | 12.3 | 21.6  | 25.7  |
| Aqueous liquor weight <sup>1</sup> | 10.5  | 10.4 | 5.1   |       |
| Total                              | 100.0 | 50.0 | 138.0 | 158.0 |

<sup>1</sup> All weights are in pounds.

Average staging temperature ° F.:

- Stage I—600–650
- Stage II—950–1,000
- Stage III—1,000–1,200
- Stage IV—1,600

As can be seen from an inspection of the data in the table, the yields of char and volatiles obtained from copyrolysis of residuum and coal are not completely additive from individual pyrolysis; whereas the oil yields are nearly additive, the char and gas yields vary. This is evident by comparing the amount of pyrolysis products obtained individually from the pyrolysis of coal and residuum and when a like amount of coal and residuum is copyrolyzed. Moreover, the data contained in this example also shows that decreasing the coal-residuum ratio tends to alter more the ratio of copyrolysis products.

**EXAMPLE 2**

The procedure of Example 1 was essentially repeated and the results thereof, along with the conditions are set forth in the table below:

TABLE II.—RUNS WITH CROWN HIGH VOLATILE B BITUMINOUS COAL AND RESIDUUM

|                              | Run   |        |       |       |
|------------------------------|-------|--------|-------|-------|
|                              | 1     | 2      | 3     | 4     |
| Dry coal weight <sup>1</sup> | 100   | 100    | 100   | 100   |
| Residuum type                | Long  | Medium | Short |       |
| Residuum weight <sup>1</sup> | 39    | 23     | 29    |       |
| Residuum to stage            | II    | II     | III   |       |
| Product yield distribution:  |       |        |       |       |
| Char weight <sup>1</sup>     | 56.6  | 57.0   | 61.0  | 62.8  |
| Oil weight <sup>1</sup>      | 19.5  | 54.5   | 41.1  | 32.8  |
| Gas weight <sup>1</sup>      | 13.8  | 14.2   | 11.9  | 19.7  |
| Liquor weight <sup>1</sup>   | 10.1  | 13.3   | 9.0   | 13.7  |
| Total                        | 100.0 | 139.0  | 123.0 | 129.0 |

<sup>1</sup> All weights are in pounds.

Average staging temperature ° F.:

- Stage I—60
- Stage II—835
- Stage III—1,200
- Stage IV—1,600

As will be noted from an inspection of the data aforesaid, the process of the invention can be run with high volatile bituminous B coal and moreover various types of residua can be used.

**6**

The identification and analysis of the coal and residua used in the examples are summarized in the following tables:

TABLE III.—ANALYSES OF COALS

| 5                                                         | Coal   | McKinley <sup>1</sup> | Crown <sup>2</sup> |
|-----------------------------------------------------------|--------|-----------------------|--------------------|
| Proximate analysis, weight percent:                       |        |                       |                    |
| Moisture                                                  | 11.6   | 10.0                  |                    |
| Volatile matter                                           | 35.5   | 34.0                  |                    |
| Fixed carbon                                              | 44.7   | 45.5                  |                    |
| Ash                                                       | 8.2    | 10.5                  |                    |
| 10 Ultimate analysis, dry basis, weight percent:          |        |                       |                    |
| Carbon                                                    | 68.5   | 67.7                  |                    |
| Hydrogen                                                  | 5.1    | 5.1                   |                    |
| Nitrogen                                                  | 1.2    | 1.7                   |                    |
| Sulfur                                                    | 0.7    | 4.0                   |                    |
| Oxygen                                                    | 15.2   | 9.9                   |                    |
| Ash                                                       | 9.3    | 11.6                  |                    |
| 15 Sieve analysis, Tyler mesh, cumulative weight percent: |        |                       |                    |
| 16                                                        | 0      | 0                     |                    |
| 28                                                        | 30.5   | 31.1                  |                    |
| 48                                                        | 58.7   | 59.2                  |                    |
| 100                                                       | 77.8   | 76.9                  |                    |
| 200                                                       | 89.0   | 87.4                  |                    |
| 325                                                       | 93.4   | 91.9                  |                    |
| Bulk density, lb./cu. ft.                                 | 46     | 47                    |                    |
| Higher heating value, dry basis, B.t.u./lb.               | 12,600 | 12,400                |                    |

<sup>1</sup> A high-volatile C bituminous coal from New Mexico.

<sup>2</sup> A high-volatile B bituminous coal from the Illinois number 6 seam.

TABLE IV.—ANALYSES OF RESIDUA

| 25                                    | Residuum type | Short | Medium | Long |
|---------------------------------------|---------------|-------|--------|------|
| Residuum description                  |               | (1)   | (2)    | (3)  |
| Gravity, ° API                        |               | 25.0  | 9.1    | 5.1  |
| Carbon residue, weight percent        |               |       |        |      |
| 30 Ultimate analysis, weight percent: |               |       |        |      |
| Carbon                                | 85.2          | 82.3  | 82.5   |      |
| Hydrogen                              | 9.2           | 10.5  | 11.3   |      |
| Nitrogen                              | 0.6           | 0.5   | 0.3    |      |
| Sulfur                                | 2.2           | 2.4   | 1.7    |      |
| Oxygen                                | 2.7           | 4.2   | 4.2    |      |
| Ash                                   | 0.1           | 0.1   | 0      |      |

35 above 1,000° F.

<sup>2</sup> Vacuum-flashed only.

<sup>3</sup> Initial boiling point around 750° F.

What is claimed is:

- 40 1. A multistage, fluid bed process of upgrading a heavy hydrocarbonaceous residue to lower boiling fractions, while simultaneously pyrolyzing finely divided coal which comprises
  - (1) in a first stage heating the finely divided coal below its fusion temperature in a first fluidized bed formed by passing an inert gasiform stream upwardly through the stage to maintain the coal in the fluidized state until about 1% to about 10% of the coal volatiles have been removed as overheads and recovering oily liquids from said overheads;
  - (2) in at least a second stage passing the so-treated coal and the heavy hydrocarbonaceous residue or a vapor into at least one other fluidized bed which is fluidized by the gaseous overhead from the subsequent stages at a temperature above that of the first bed and below the fusion point of the solids fed to that stage for a time sufficient to remove nearly all of the volatiles condensable to other liquids;
  - (3) in a final stage passing the thus treated coal and residue into a final fluidized bed which is fluidized by an oxygen containing gas at a still higher temperature to substantially devolatilize the coal and residue; and
  - (4) recovering the oily liquid from all stages subsequent to the first stage, from the overhead of the second stage.
- 45 2. A multistage, fluid bed process of upgrading a heavy hydrocarbonaceous residue to lower boiling fractions, while simultaneously pyrolyzing particles of high volatile C bituminous coal which comprises
  - (1) in a first stage heating the coal to a temperature of about 600° F. to about 650° F. in a first fluidized bed formed by passing an inert gasiform stream upwardly through the stage to maintain the coal in the fluidized state until about 1% to about 10% of
- 50 55 60 65 70 75

- the coal volatiles have been removed as overheads and recovering oily liquids from said overheads; (2) passing the thus treated coal and vaporized hydrocarbonaceous residue into a second bed which is fluidized by the gaseous overheads from the subsequent stages at a temperature of 950° F. to 1000° F. for a time sufficient to remove substantial amounts of volatiles from the products; (3) passing the thus partially pyrolyzed products along with a further quantity of hydrocarbonaceous residue into a third fluidized bed which is fluidized by the gaseous overheads from the subsequent stages, at a temperature of 1000° F. to 1200° F. for a time sufficient to reduce the remaining volatiles in the coal and hydrocarbonaceous residue condensable to oily liquid to no more than about 1%; (4) passing this product of pyrolyzed coal and hydrocarbonaceous residue into a fourth fluidized bed which is fluidized by an oxygen containing gas maintained at a temperature of 1500° F. to 1600° F. to substantially devolatilize the char; and (5) recovering the condensables from the overheads of all stages subsequent to the second stage from the overhead of the second stage.
3. The method of claim 1 in which oxygen containing gas is fed into the fourth fluidized bed to react the char to provide heat and the overheads are fed countercurrently to the third and second stages to heat them.
4. A multistage, fluid bed process of upgrading a heavy hydrocarbonaceous residue to lower boiling fractions while simultaneously pyrolyzing particles of high volatile B bituminous coal which comprises
- (1) in a first stage heating the coal to a temperature of about 650° F. in a first fluidized bed formed by passing an inert gasiform stream upwardly through the stage to maintain the coal in the fluidized state until about 1% to about 10% of the coal volatiles have been removed as overheads and recovering oily liquid from said overheads;
  - (2) passing the thus treated coal into a second stage

5

10

15

20

25

30

35

40

- which is fluidized by the gaseous overheads from the subsequent stages at a temperature of 800° F. to 900° F. for a time sufficient to remove substantial amounts of volatiles; (3) passing the thus partially pyrolyzed coal particles along with the hydrocarbonaceous residue into a third fluidized bed which is fluidized by the gaseous overheads from the subsequent stages at a temperature of 1000° F. to 1200° F. for a time sufficient to reduce the remaining volatiles in the coal and hydrocarbonaceous residue condensable to oily liquid to no more than about 1%; (4) passing this product of pyrolyzed coal and hydrocarbonaceous residue into a fourth fluidized bed which is fluidized by an oxygen containing gas maintained at a temperature of 1500° F. to 1600° F. to substantially devolatilize the char; and (5) recovering the condensables from the overheads of all stages subsequent to the second stage from the overhead of the second stage.

5. The method of claim 3, wherein char is recycled from the final stage to a preceding stage.

#### References Cited

##### UNITED STATES PATENTS

|            |         |          |       |        |
|------------|---------|----------|-------|--------|
| Re. 24,574 | 12/1958 | Welinsky | ----- | 201—31 |
| 2,955,077  | 10/1960 | Welinsky | ----- | 201—31 |
| 2,982,701  | 5/1961  | Scott    | ----- | 208—11 |
| 3,011,953  | 12/1961 | Foch     | ----- | 201—44 |

##### FOREIGN PATENTS

|         |        |               |       |        |
|---------|--------|---------------|-------|--------|
| 413,927 | 7/1934 | Great Britain | ----- | 201—23 |
| 785,994 | 1/1957 | Great Britain | ----- | 201—23 |

35 WILBUR L. BASCOMB, JR., Primary Examiner

D. EDWARDS, Assistant Examiner

U.S. CL. X.R.

201—31, 44, 28; 208—127

UNITED STATES PATENT OFFICE  
CERTIFICATE OF CORRECTION

Patent No. 3,565,766 Dated February 23, 1971

Inventor(s) Ralph Tracy Eddinger and John F. Jones

It is certified that error appears in the above-identified patent and that said Letters Patent are hereby corrected as shown below:

Column 3, line 2, "by" should read --to--.

Column 4, line 15, "fed" should read --feed--.

Column 4, line 50, "are" should be inserted at end of line.

Column 5, line 67, "60" should read --600--.

Signed and sealed this 28th day of March 1972

(SEAL)

Attest:

EDWARD M. FLETCHER, JR.  
Attesting Officer

ROBERT GOTTSCHALK  
Commissioner of Patents